

Aug. 11, 1931.

J. R. CAIN ET AL

1,818,379

PROCESS FOR THE MANUFACTURE OF METALLIC SHEETS

Filed Dec. 2, 1927



INVENTOR.  
John R. Cain  
BY *Robert Youngblood*  
Ollie *Allen* ATTORNEYS

## UNITED STATES PATENT OFFICE

JOHN R. CAIN, OF WASHINGTON, DISTRICT OF COLUMBIA, AND GIBSON YUNGBLUT, OF DAYTON, KENTUCKY, ASSIGNORS TO THE RICHARDSON COMPANY, OF LOCKLAND, OHIO, A CORPORATION OF OHIO

## PROCESS FOR THE MANUFACTURE OF METALLIC SHEETS

Application filed December 2, 1927. Serial No. 237,295.

Our invention has to do with processes of forming metallic sheets directly by electrolytic means. In such processes metallic sheets are deposited from a suitable electrolyte by the action of an electric current, upon a conducting surface which forms the cathode of an electrolytic cell. A number of such processes have been proposed and some of them are in practical operation.

10 The deposition of metal upon a rotating cylindrical cathode from which the deposit is continuously stripped, has been proposed. Electrolytic sheet copper is made to-day by electrodepositing copper upon prepared cathode blanks the surfaces of which have been sulphided or otherwise treated so that the deposit may be more or less readily removed therefrom.

15 In the manufacture of thin sheets or foils, particularly of the precious metals, it has been proposed to plate the precious metal upon a cathode blank of base metal, which may be in the form of a sheet or strip or the like, and subsequently to remove the base metal from the precious metal by the use of a chemical reagent which will selectively attack it.

20 All of these processes, however, involve either a mechanical stripping, which is cumbersome, expensive and uncertain, or a chemical stripping which results in the destruction of the cathode blank.

25 In application filed on August 19th, 1927, by the present applicants, Serial No. 214,194, the method of forming electrolytic sheets is set forth, wherein a rolling or elongating step is relied upon to increase the cathode area so as to produce not only a finished or semi-finished end product of the operation, but also a piece which will serve as the cathode in a continuation of the process.

30 It is the object of the present invention to utilize in a bimetallic sheet-forming operation a method of continuously regenerating the cathode blanks so that the process becomes a continuous one and is not subject to an outside source of supply for cathode blanks. We accomplish our object by that certain series of steps which will be herein-50 after specifically pointed out in a typical

example, and in which the inherent novelty will be set forth in the claims that follow.

Referring to the drawings:

Figure 1 is diagrammatic inasmuch as the mechanisms by which the several steps are accomplished are well known to those skilled in the electrolytic and metal-working arts.

Figures 2 to 7 are illustrative of the several stages of treatment suitably labeled.

Briefly stated, our process consists in starting with a cathode blank of a metal which we will designate as 1. This is placed in an electrolytic cell A and forms the cathode thereof.

The electrolyte B is a solution of a salt of a metal dissimilar to the metal of the cathode blank 1, and the anode C may advantageously contain the same metal as that which the electrolyte contains, though insoluble anodes may of course be used in the process. The action of a source of electrical energy D connected to the anode and the cathode blank is to cause a deposit of metal 2 to be laid down upon the cathode blank 1.

We continue the electrolytic action in the cell A until the thickness of the deposited metal sheet is also twice that required in the finished product.

The bimetallic article 1-2 is now removed from the electrolytic bath, washed as at F and subjected to one or more passes through a rolling mill E, with such intervening annealings as may be required by the nature of the metals and the amount of reduction contemplated. In this rolling operation we reduce the metallic composite 1-2 at least to one-half its thickness, and we may, if desired, reduce it further, as will be apparent later. In this rolling operation the length will obviously be at least doubled.

We next sever as by shear G the rolled metallic article into two parts (assuming that we have doubled its length and decreased its thickness by one-half), and we designate the two parts thus formed as portions 1a-2a and 1b-2b. Both of these bimetallic articles are placed in an electrolytic stripping cell H containing as an electrolyte a solution of a salt of the metal 1, of such characteristics that under electrolytic conditions the metal

2 will not be attacked, but the metal 1 will be dissolved at the anode and deposited at the cathode.

We make one of our bimetallic articles the 5 anode and the other the cathode, facing metal portions 1a and 1b toward each other, and utilize through suitable connection a source of electrical energy indicated at I. The result of the electrolytic action will be to dissolve the metal from one bimetallic article, 10 and to deposit an equivalent amount of metal upon the other bimetallic article which we have made the cathode of the couple.

The end product of the anode in this electrolytic process will be a finished sheet of metal 2. This finished sheet will be of the required or single thickness. The end product of the cathode in the cell H will be a bimetallic article consisting of a single thickness of 20 the metal 2 and a double thickness of the metal 1, and we have designated this at 4. It will be obvious that this can be returned to the electrolytic cell A to receive a further deposit of the metal 2 and the process will thus 25 be continuous and precisely identical with the steps hitherto described except that the action of the electric current in the cell A need be continued only long enough to deposit a single thickness of the metal 2 on the composite blank 4, since one thickness is there 30 already.

We will now give as a typical example a process of manufacturing thin iron sheets upon a prepared cathode blank of copper. 35 We start as above indicated with a copper cathode blank which will be a smooth rolled sheet of soft copper of the size of the required finished iron sheet and of a convenient thickness, which may be .04". Our electrolyte in the electrolytic cell A will be a hot 40 neutral ferrous chloride electrolyte containing approximately 100 grams metallic iron per liter, and the electrolytic process which we propose to use is to employ an anode formed of iron sulphide 45 together with other conditioning means, and a filtration system for the electrolyte which keeps down hydrogen ion concentration to a negligible amount, and keeps the electrolyte 50 free from sediment.

The result of this practice is to keep the said bath "in condition" so that the iron electrodeposited therefrom will be soft, malleable and ductile, and if the current density 55 is maintained at the proper values, of a fine grained nature.

Through the action of a suitable source of electrical energy we deposit iron upon the copper cathode blank until its thickness is 60 .04" or somewhat greater. The resultant bimetallic article will therefore be .08" in thickness or thereabouts.

We then remove it from the bath and after 65 washing pass it through cold rolls until its length is doubled and its thickness again re-

duced to .04". The product after rolling will consist therefore of a layer of copper .02" in thickness and a layer of iron also .02" in thickness. The softness of the iron deposited in the electrolytic process which we prefer 70 to use, we have found to be such that in the reduction of the composite blank by rolling the iron and copper will be reduced equally. We know of no other way of obtaining a soft iron deposit than following generally the 75 method above referred to or modifications thereof. This method is set forth in this application, however, as a preferable method.

Such intervening annealings as may be necessary will be within the knowledge of the skilled operator to perform; but inasmuch as the copper, upon rolling, tends to harden up much more rapidly than the iron, it is frequently possible to use in an annealing step a temperature such as will anneal the copper and not the iron, or anneal the copper more 80 than the iron. We have thus found it possible to use in annealing a bath of hydrocarbon oil heated to about 400° centigrade, through 85 which the strip is passed slowly, or in which it is submerged in any desired way, which 90 will soften the copper without oxidizing and with a reducing action leaving the surface bright, but will have very little effect upon the iron. It will be further obvious that in 95 connection with the rolling operation the operator will do such trimming of the metallic composite as may be necessary and that the thickness of the various deposits will have 100 to take into account any necessary trim.

We next sever our composite article into two parts and place them both in an electrolytic cell H containing a solution of cyanide of copper. Two bimetallic pieces are placed in the bath with the copper faces toward each other. One of them is made the anode and the other the cathode, and suitable connections made to a source of electrical energy, under the action of which the copper will 105 be dissolved from the face of the iron on the anode and deposited upon the copper face of the cathode.

At the end of the electrolytic stripping operation the anode will consist of the finished iron sheet .02" in thickness, one face of which 110 will have been electrodeposited against a rolled face of the copper blank and the other face of which will have been rolled in the rolling operation described above, and also 115 trimmed. It therefore will be a smooth and 120 polished finished article on both sides.

The cathode blank removed from the stripping cell will consist of a double thickness of copper and a single thickness of iron. After 125 washing, it may be transferred directly back to the electrolytic cell A for a further deposit of iron on the iron face thereof, although if desired, it may be passed through cold rolls, before being returned to the ferrous chloride electrolytic cell.

Having thus described our invention, what we claim as new and desire to secure by Letters Patent, is:—

1. That process of forming an electrode-deposited metallic object, which consists in plating the object onto a cathode, elongating the cathode to at least twice its original length, severing the cathode to form an article of the desired shape, and plating the cathode metal from said object back onto the remainder of the original cathode, thus forming a new cathode having original thickness of the cathode metal and half of the plated thickness of the same metal as the metallic object, and then plating on the new cathode with the metal of the object to form a new blank for elongating, for the purpose described.

2. That process of forming electrolytic metal sheets, which consists in plating a desired metal on a cathode sheet, elongating the sheet to at least twice its original length, severing the cathode to form a sheet of the desired area, plating the cathode metal from the severed body back onto the cathode metal of the remainder of the elongated cathode, thus making a new cathode, and then plating the desired metal onto the portion of the new cathode blank which is of that metal, for the purpose described.

3. That process of forming electrolytic metal sheets, which consists in plating a desired metal on a cathode sheet, elongating the sheet to at least twice its original length, severing the cathode to form a sheet of the desired area, plating the cathode metal from the severed body back onto the cathode metal of the remainder of the elongated cathode, thus making a new cathode, and then plating the desired metal onto the portion of the new cathode blank which is of that metal, for the purpose described, said elongating being accomplished by cold rolling.

4. That process of forming iron sheets or foils, which consists in plating iron onto a copper sheet, cold rolling the plated body and cutting from it a piece of a desired area, plating the copper from the severed piece back onto the copper of the remainder of the elongated cathode blank making a new cathode, then plating iron on the iron portion of the new cathode, for the purpose described.

5. That process of forming electrolytic iron sheets, which consists in plating iron on a sheet of another metal, elongating the composite sheet, electrolytically stripping the other metal from the iron by plating it onto a strip of metal and employing said strip of metal as cathode material in a subsequent plating operation.

6. That process of forming electrolytic metal pieces, which consists in plating said metal on a piece of another metal which is alike in shape to the product to be produced, working the composite piece thus formed and stripping the other metal off by plating it

onto a piece of the same shape as the piece to be stripped, and employing said piece onto which the second plating is applied as cathode material in a subsequent plating operation.

7. That process of forming electrolytic metal sheets, which consists in plating the metal on a starting sheet of another metal, working the composite sheet thus produced and electrolytically stripping the other metal from the sheet by plating it onto a piece of metal which is the result of a working of a sheet such as the starting sheet, and using said secondly plated sheet as a cathode for a second plating operation.

8. That process of forming electrolytic iron pieces, which consists in plating iron onto a piece of copper, working the composite piece thus formed and stripping the copper away from the plated piece by plating off the copper onto a piece of copper and employing said piece of copper in a subsequent plating operation.

JOHN R. CAIN.  
GIBSON YUNGBLUT.

90

95

100

105

110

115

120

125

130